

Nov. 11, 1930.

H. M. NAUGLE ET AL

1,781,123

METHOD OF COLD ROLLING AND COILING STRIPS

Original Filed Sept. 23, 1924 3 Sheets-Sheet 1



Inventors  
H. M. Naugle  
and A. J. Townsend  
By  
Grease and Bond Attorneys

Nov. 11, 1930.

H. M. NAUGLE ET AL

1,781,123

METHOD OF COLD ROLLING AND COILING STRIPS

Original Filed Sept. 23, 1924 3 Sheets-Sheet, 2



Fig. 5.

Inventors  
H. M. Naugle and  
A. J. Townsend  
By

Greene and Bond, attorneys

Nov. 11, 1930.

H. M. NAUGLE ET AL

1,781,123

METHOD OF COLD ROLLING AND COILING STRIPS

Original Filed Sept. 23, 1924 3 Sheets-Sheet. 3

*Fig. 4.*



*Fig. 5.*



*Fig. 6.*

*Fig. 7.*



Inventors

H. M. Naugle

and A. J. Townsend

By Spear and Bond Attorneys

SPEED-LOAD CHARACTERISTIC CURVES

1. DIFFERENTIALLY WOUND COMPOUND MOTOR
2. SHUNT WOUND MOTOR
3. CUMULATIVELY WOUND COMPOUND MOTOR

## UNITED STATES PATENT OFFICE

HARRY M. NAUGLE AND ARTHUR J. TOWNSEND, OF CANTON, OHIO, ASSIGNEES, BY MESNE ASSIGNMENTS, TO THE AMERICAN ROLLING MILL COMPANY, OF MIDDLE-TOWN, OHIO, A CORPORATION OF OHIO

## METHOD OF COLD ROLLING AND COILING STRIPS

Continuation of application Serial No. 739,302, filed September 23, 1924. This application filed April 28, 1927. Serial No. 187,186.

The invention relates to the reduction of strips of steel and the like to a finishing gauge by cold rolling and coiling the same; the object of the improvement is to impede or 5 preclude the formation of imperfections in the strip and to remove such imperfections as may be formed therein; and this application is a continuation of our pending application filed September 23, 1924, Serial No. 739,302, 10 for the same invention.

Each time a strip is reduced in thickness between cold rolls, the unavoidable variation in the pressure of the rolls from one side toward the other side of the strip, which may 15 be caused by an unequal pressure adjustment of the ends of the rolls, or an inaccurate or uneven turning or wearing of the faces thereof, or an unequal heating of the body of the rolls, results in giving the strip a lateral camber, and sometimes a fullness in the middle 20 portion which causes it to buckle between the edges thereof.

Furthermore, the elongation of a strip by 25 the reducing action of successive mills, causes a looping of the strip between successive mills and between the last mill and the coiler, and a consequent bending or distortion of the strip.

And finally, the presence of the imperfections referred to, and especially, the presence 30 of long loops in the strip, limits the amount of reduction which can be made by one of the mills, and requires mills to be operated at a comparatively low rate of speed, thus limiting 35 the productive capacity of the apparatus.

The present improvement may be carried 40 out by independently driving each successive tandem mill and the coiling drum at an increased peripheral speed from that of the previous mill, and regulating the grip and the speed of same so that the strip is automatically stretched between successive mills and the coiler to give it a tension greater than the elastic limit of the metal, which will not only 45 elongate the strip and straighten the bends and buckles and the camber there may be therein; but will also prevent, to a certain extent, the formation of such defects by the cold roll reducing operations.

50 In this manner the strip is constantly kept

in a tension greater than the elastic limit of the metal throughout all the operations, which not only prevents, either wholly or in part, the formation of the described defects, and precludes the accumulation of such defects as may be formed, but also acts to remove the same when they have been formed.

To this end, it is necessary that each successive reducing mill and the coiler drum, shall grip and pull the strip with such a positive engagement as will constantly give the required tension greater than the elastic limit of the metal for the preventive and corrective operations upon the strip, so that the shorter sides and portions of the strip will be elongated to the full length of all other portions thereof, and will remain set at such full length against any elastic reaction to a shorter length.

Such a result cannot be attained by the tension resulting from the engagement of finishing cold rolls which do not have enough pressure to materially reduce the thickness of the strip; because such cold rolls cannot grip and pull the strip with sufficient force to remove all the fullness and camber therein, and much less to prevent the formation and accumulation of such defects.

This is because cold rolled steel has a very high tensile strength or elastic limit as compared with hot rolled steel. The tensile strength of hot rolled steel strips in the finishing passes may be as low as 10,000 pounds per square inch depending upon the temperature; while the tensile strength of cold rolled steel strips in the finishing passes, may be as high as 90,000 pounds per square inch.

Nor can such a result be attained by a differential tension control of the peripheral speed of successive mills, which merely equalizes the work of the rolls for reducing the thickness of a strip; for the reason that the tension required for such purpose is not sufficient to stretch and straighten the strip for elongating the same to attain the results herein set forth.

Furthermore, such a result cannot be attained by merely pulling or stretching the strip with a tension approaching or even at about the elastic limit of the metal, because

55

60

65

70

75

80

85

90

95

100

the elastic limit of the metal in the strip must be fully exceeded to elongate any portion or all of the same, and the elastic tendency of the metal which has been elongated to contract and return to its original condition must be entirely overcome, to accomplish the purpose of the present improvement.

And finally, the differential speed control of each successive mill and the coiling drum must be automatically regulated so that while constantly maintaining a tension exceeding the elastic limit of the metal, which is required for stretching, straightening and setting the structure of the strip, the tension will not exceed the ultimate strength of the metal and thereby strain or sever the strip.

The object of the present invention may be attained by providing each successive mill and the coiler drum with a cumulatively wound compound electric motor; and by increasing the series winding as compared with the shunt winding ordinarily used in such a motor, so as to cause the motor to respond more readily to slight variations in the load and to modify the speed in accordance therewith, thereby maintaining the necessary tension for straightening the strip by elongating the same without tearing it apart.

The invention is illustrated in the accompanying drawings, forming part hereof, in which—

Figure 1 is an outline plan view of a series of tandem cold rolling mills and a coiling drum, showing the roll housing in section;

Fig. 2, an enlarged elevation section of two adjacent mills, each on line 2—2, Fig. 1;

Fig. 3, a similar section of the last mill of the series and an end view of the coiling drum;

Fig. 4, a conventional diagrammatic view of a cumulatively wound compound electric motor;

Fig. 5, a conventional section of a field core showing a one-half winding of the series coil;

Fig. 6, a similar view showing a one and one-half winding of a series coil; and

Fig. 7, a diagrammatic view showing the speed-load characteristic curves of different types of motors.

Similar numerals refer to similar parts throughout the drawings.

The successive rolling mills 10, 10<sup>a</sup>, 10<sup>b</sup> and 10<sup>c</sup> of a tandem series and the coiling drum 11' at the end of the series, are driven by individual electric motors 11, 11<sup>a</sup>, 11<sup>b</sup>, 11<sup>c</sup> and 11<sup>d</sup>; and for the purpose of the present invention these motors are made of the cumulatively wound compound type, as diagrammatically shown in Fig. 4.

The speed load characteristic curve of such a motor is shown at 13 in Fig. 7, as compared with the corresponding curve 14 of a shunt wound motor and the corresponding curve 15 of a differentially wound compound

motor; and as shown in Fig. 7, the percentage of speed decreases quite rapidly as the percentage of load increases in a cumulatively wound motor, thereby causing the speed thereof to respond very readily to differences in the load.

In order to increase the responsive action of such a motor, for the purpose of the present invention, it is preferred to increase the winding of the series coil from the half winding used in common practice, as shown in Fig. 5, to a one and one-half winding, as shown in Fig. 6; which modification of the winding has proved very satisfactory in a standard of 250 H. P., 250 volt compound wound adjustable speed motor.

The operation of tandem cold rolling mills for reducing the thickness of a steel strip in accordance with common practice, from an initial thickness of about one hundred and nine thousandths (.109) of an inch produced by hot rolling processes, to a final thickness of about thirty-two thousandths (.032) of an inch, may be described briefly as follows:—

A first roughing operation may be carried out by a series of four stands of cold rolls, with or without a coiler at the delivery end thereof, by which the thickness of the strip is reduced from about .109 to about .062 of an inch; after which the strip is preferably annealed, which may be done in an ordinary annealing furnace.

A second roughing operation may then be carried out by a similar series of cold rolls, which is preferably provided with a coiling device at the delivery end, as illustrated in Fig. 1, by which the thickness of the strip is reduced from about .062 to about .036 of an inch; it being understood that each stand of cold rolls performs its relative proportion of the reducing process, as the strip passes between the rolls thereof.

A levelling operation may then be carried out by a single stand of cold rolls with or without a coiler, by which operation the thickness of the strip is reduced from about .036 to about .035 of an inch; after which the strip may be again annealed in an ordinary annealing furnace.

And finally, a finishing skin rolling operation may be carried out by a single stand of cold rolls, which is preferably associated with a coiling drum; by which operation the thickness of the strip is reduced from about .035 to about .032 of an inch.

For the purpose of carrying out the present improvement, the motor of each successive stand of rolls, and of the coiler when the same is used, is set or adjusted to normally rotate each stand of rolls and the coiler at a greater peripheral speed than the next previous stand of rolls, so as to constantly pull the strip with an elongating stretching tension beyond the elastic limit but within the ultimate strength.

of the metal, from the delivery side of each stand of rolls.

The inherent characteristics of the motors when wound as described, causes each motor 5 to automatically increase its speed when the strip tension load thereon is decreased, and vice versa; so that an elongating stretching tension as aforesaid, is constantly maintained upon the strip throughout its length from 10 the delivery side of each stand of rolls to the next succeeding stand of rolls or to the coiling drum, as the case may be.

The improved method of reducing a strip by one or more cold-rolling mills and a coiler, 15 combined with motors as described, is illustrated in Figs. 2 and 3, wherein the course from one mill to another or to the coiler, of a strip or sheet stretched and elongated by constant tension is shown in full lines at 16 or 20 16'; while the tortuous course from one mill to another or to the coiler, of a strip or sheet which is not stretched by tension, is shown in broken lines at 16<sup>a</sup> or 16<sup>a'</sup>.

When an elongating stretching tension is 25 constantly maintained upon the metal in a strip passing from one mill to another or to a coiler, the same not only serves to straighten any camber and to flatten any fullness there may be therein, but acts to avert, more or 30 less, the formation of such defects by the reducing pressure of the rolls.

And, it has been found, furthermore that the constant tension upon the strip not only 35 enables the cold rolling and coiling apparatus to be operated at a much higher speed, but permits a greater reduction to be made in the thickness of the strip by each pass between the rolls; thus greatly increasing the productive capacity of the apparatus, which 40 can, moreover, be used to reduce strips of more than ordinary width, say up to some thirty or forty or more inches, when operated in a manner to carry out the improved method described herein.

45 We claim:—

The method of reducing the thickness of strips of steel and the like by tandem stands of rolls, which consists in constantly maintaining an elongating stretching tension 50 greater than the elastic limit but less than the ultimate strength of the metal in the strip on both sides of each successive stand of rolls, to straighten and set the structure of the strip; the pull on the strip extending between the successive stands of rolls being 55 caused by action of the succeeding stand of rolls upon the strip between it and the previous stand of rolls.

HARRY M. NAUGLE.  
ARTHUR J. TOWNSEND.